

# UNITED STATES PATENT OFFICE.

ARTHUR SAMUEL O'NEIL, OF WILMINGTON, DELAWARE, ASSIGNOR TO E. I. DU PONT DE NEMOURS AND COMPANY, OF WILMINGTON, DELAWARE, A CORPORATION OF DELAWARE.

## PROCESS OF PRODUCING PROPELLENT EXPLOSIVES.

1,311,909.

Specification of Letters Patent. Patented Aug. 5, 1919.

No Drawing.

Application filed August 17, 1916. Serial No. 111,451.

*To all whom it may concern:*

Be it known that I, ARTHUR SAMUEL O'NEIL, of Wilmington, Del., in the county of New Castle, and in the State of Delaware, have invented a certain new and useful Improvement in Processes of Producing Propellant Explosives; and I do hereby declare that the following is a full, clear, and exact description thereof.

10 My invention relates to improvements in processes of producing propellant powders.

My invention relates particularly to a process of producing smokeless powders so as to provide a surface treatment to produce what is known as progressive powders, that is to say, powders adapted to produce a lower initial pressure without lowering the velocity of the projectile. My invention is applicable to the production of various kinds of rifle and cannon powders.

20 The object of my invention is to provide a process for the treatment of powder by which many of the disadvantages of previous powders of this type may be avoided.

25 More particularly the object of my invention is to provide a process of producing a powder of this character by applying to the surface of powder grains, as for example the grains of nitrocellulose powder a deterrent material, which is a solvent of the explosive contained in the powder grains, so that it may be caused to penetrate the powder grains, and which is substantially non-volatile and which further provides on the surface of the 30 grains an explosive of sufficient potential to obtain satisfactory ignition.

35 A further object of my invention is to provide a process of this character by applying a material to the surface of the 40 powder grains which has substantially no odor and which is so slightly volatile that the powder produced in connection with my invention may be stored at the temperature to which powders are ordinarily subjected 45 without producing any substantial ballistic change.

Previously, in order to apply coating materials to powder grains it has been customary either to dissolve the material in a 50 suitable solvent and spray the solution onto the powder while the latter is stirred, after which the solvent is evaporated or the coating material has been applied in the form of a dry powder by the use of a glazing or

tumbling barrel followed by heat treatment. 55 When smokeless powder is surface coated with various materials in the above described manner, there results little improvement in the progressive burning of the powder, and there is produced considerable 60 tendency to hang fire, particularly if the materials used for coating are deterrent materials of a low explosive or non-explosive order, and difficult of ignition. It has been found, however, that many substances for 65 coating purposes, which would be highly desirable because of their stability, low volatility, absence of odor, and lack of injurious action on the powder are unsuitable because of their high melting point. 70

A further object of my invention is therefore, to make use of such substances in coating powder in such a way as to lower their melting point, thus avoiding the objections to their use due to their high melting point. 75

While my invention is capable of being carried on in many different ways, for the purpose of illustration, I shall describe only one form of my invention hereinafter.

For example, a quantity of nitrocellulose 80 powder in the form of grains is introduced into a revolving barrel, provided with means for heating the same. A mixture of a nitro-hydrocarbon, such as dinitrotoluene with camphor added thereto, or with diphenyl-85 amin also added thereto, is introduced into the barrel. The dinitrotoluene may be any of the several isomers or it may be a mixture of isomers formed by the direct nitration of toluene; but I prefer to use merely 90 pure dinitrotoluene, which is usually described as the 1, 2, 4 isomer (c. p. dinitrotoluene). The mixture of dinitrotoluene, camphor and diphenylamin may be in the proportions of 84 parts of dinitrotoluene, 16 95 parts of camphor and 4 parts of diphenylamin, the melting point of the mixture being in the neighborhood of 65° C.—whereas the 1, 2, 4 isomer of dinitrotoluene melts at about 70.5° C. This mixture when 100 warmed is partially liquefied and is mixed with the powder grains in the rotating barrel for about half an hour to insure a uniform coating. The powder may be allowed to stand over night to allow the mixture 105 which is a partial solvent to penetrate the grains. The temperature of the barrel is then gradually raised to 65° C. and the bar-

rel rotated from one to one and a half hours. The excess of camphor volatilizes and the dinitrotoluene with some of the camphor impregnates the grains. The powder grains, if allowed to cool in this condition would adhere to one another and a small amount of graphite suitable for glazing smokeless powder is added and the mixing is continued until the powder becomes dry, which 5 takes about twenty minutes. An additional amount of graphite is then added and the glazing of the powder is completed. The graphite not only serves to glaze the powder, but also serves to separate the powder grains 10 and permit the individual grains to become effectively impregnated with the dinitrotoluene mixture. The powder grains so treated no longer adhere to one another, the individual grains have been effectively impregnated with the dinitrotoluene. The 15 finished powder is capable of producing an increased velocity with the same or a lower pressure than in the case of the original powder before being subjected to the above 20 treatment.

While I have described my invention above in detail, I wish it to be understood that many changes may be made therein, without departing from the spirit of my invention.

I claim:—

1. The process which comprises applying to nitrocellulose powder grains a nitro-hydrocarbon having a solvent action on the nitrocellulose grains, said nitro-hydrocarbon containing an aromatic compound which lowers the melting point thereof, and heating the materials to a temperature materially below the melting point of the nitro-hydrocarbon used.

2. The process which comprises applying to nitrocellulose powder grains a nitro-hydrocarbon having a solvent action on the nitrocellulose grains, said nitro-hydrocarbon containing an aromatic compound which lowers the melting point of the nitro-hydrocarbon, and heating the materials to a temperature of approximately 65° C.

3. The process which comprises applying to nitrocellulose powder grains a nitro-hydrocarbon having a solvent action on the nitrocellulose grains, said nitro-hydrocarbon containing camphor which lowers its melting point, and then heating the mixture.

4. The process which comprises mixing nitrocellulose powder grains with a nitro-

hydrocarbon having a solvent action on the nitrocellulose grains, said nitro-hydrocarbon containing camphor and diphenylamin which lowers its melting point, and heating 60 the mixture during the mixing operation.

5. The process which comprises applying to nitrocellulose powder grains a mixture at least partially liquefied of dinitrotoluene and camphor.

6. The process which comprises applying to nitrocellulose powder grains a mixture at least partially liquefied of dinitrotoluene, camphor and diphenylamin.

7. The process which comprises applying to nitrocellulose powder grains a mixture at least partially liquefied of 1, 2, 4 dinitrotoluene and camphor.

8. The process which comprises applying to nitrocellulose powder grains a mixture at least partially liquefied of 1, 2, 4 dinitrotoluene, camphor and diphenylamin.

9. The process which comprises applying to nitrocellulose powder grains a mixture at least partially liquefied of dinitrotoluene 80 and a stabilizer for nitrocellulose.

10. The process which comprises applying to nitrocellulose powder grains a mixture at least partially liquefied of dinitrotoluene, camphor and a stabilizer for nitrocellulose.

11. The process which comprises applying to nitrocellulose powder grains a mixture of 84 parts dinitrotoluene, 16 parts camphor and 4 parts diphenylamin to impregnate the 90 surface of the grains with dinitrotoluene.

12. The process which comprises mixing nitrocellulose powder grains with a mixture of dinitrotoluene, camphor and diphenylamin, warming the mixture to partially liquefy the dinitrotoluene and continuing the mixing until the powder grains are coated with the partially liquefied dinitrotoluene, gradually increasing the temperature of the mixture to approximately 65° centigrade, to 100 completely liquefy the dinitrotoluene and continuing the mixing for a substantial period to promote a reaction between the dinitrotoluene and the nitrocellulose grains, and drying and glazing the grains.

In testimony that I claim the foregoing I have hereunto set my hand.

ARTHUR SAMUEL O'NEIL.

Witnesses:

EDWIN F. STIMPSON,  
VICTOR E. COMEGYS.